

Nov. 2, 1965

E. E. DASCHER  
METHOD OF COATING METAL FOILS WITH A POLYMERIZABLE  
RESINOUS COATING

3,215,558

Filed Feb. 16, 1959

17 Sheets-Sheet 1



EDWARD E. DASCHER

INVENTOR.

Fig. 1

BY *Edward E. Dascher*

ATTORNEY

Nov. 2, 1965

E. E. DASCHER

3,215,558

METHOD OF COATING METAL FOILS WITH A POLYMERIZABLE  
RESINOUS COATING

Filed Feb. 16, 1959

17 Sheets-Sheet 2



Nov. 2, 1965

E. E. DASCHER  
METHOD OF COATING METAL FOILS WITH A POLYMERIZABLE  
RESINOUS COATING

3,215,558

Filed Feb. 16, 1959

17 Sheets-Sheet 3

Fig. 3



Fig. 4



Fig. 5



Fig. 4a



Fig. 8



Fig. 7



INVENTOR.  
EDWARD E. DASCHER

BY

Edward Dascher  
ATTORNEY

Nov. 2, 1965

5 E. E. DASCHER 3,21  
METHOD OF COATING METAL FOILS WITH A POLYMERIZABLE  
RESINOUS COATING

3,215,558

Filed Feb. 16, 1959

17 Sheets-Sheet 4



EDWARD E. DASCHER  
INVENTOR.

BY *Howard Meacham*  
ATTORNEY

Nov. 2, 1965

5 E. E. DASCHER 3,2  
METHOD OF COATING METAL FOILS WITH A POLYMERIZABLE  
RESINOUS COATING

3,215,558

Filed Feb. 16, 1959

17 Sheets-Sheet 5



EDWARD E. DASCHER  
INVENTOR.

BY  
*Alfred, Alfred*  
ATTORNEY

Nov. 2, 1965

E. E. DASCHER

3,215,558

METHOD OF COATING METAL FOILS WITH A POLYMERIZABLE  
RESINOUS COATING

Filed Feb. 16, 1959

17 Sheets-Sheet 6



Nov. 2, 1965

E. E. DASCHER  
METHOD OF COATING METAL FOILS WITH A POLYMERIZABLE  
RESINOUS COATING

3,215,558

Filed Feb. 16, 1959

17 Sheets-Sheet 7



Nov. 2, 1965

E. E. DASCHER

3,215,558

METHOD OF COATING METAL FOILS WITH A POLYMERIZABLE  
RESINOUS COATING

Filed Feb. 16, 1959

17 Sheets-Sheet 8



EDWARD E. DASCHER  
INVENTOR.

BY *Edward Dascher*

ATTORNEY

Nov. 2, 1965

55 E. E. DASCHER 3,2  
METHOD OF COATING METAL FOILS WITH A POLYMERIZABLE  
RESINOUS COATING

3,215,558

Filed Feb. 16, 1959

17 Sheets-Sheet 9



INVENTOR.  
EDWARD E. DASCHER

BY *Harold Meacham*  
ATTORNEY

Nov. 2, 1965

E. E. DASCHER  
METHOD OF COATING METAL FOILS WITH A POLYMERIZABLE  
RESINOUS COATING

3,215,558

Filed Feb. 16, 1959

17 Sheets-Sheet 10



Nov. 2, 1965

E. E. DASCHER

3,215,558

METHOD OF COATING METAL FOILS WITH A POLYMERIZABLE  
RESINOUS COATING

Filed Feb. 16, 1959

17 Sheets-Sheet 11



Nov. 2, 1965

5 E. E. DASCHER 3,2  
METHOD OF COATING METAL FOILS WITH A POLYMERIZABLE  
RESINOUS COATING

3,215,558

Filed Feb. 16, 1959

17 Sheets-Sheet 12



EDWARD E. DASCHER  
INVENTOR.

BY *Reuben Deuchn*  
ATTORNEY

Nov. 2, 1965

E. E. DASCHER

3,215,558

METHOD OF COATING METAL FOILS WITH A POLYMERIZABLE  
RESINOUS COATING

Filed Feb. 16, 1959

17 Sheets-Sheet 13



Fig. 25

INVENTOR.  
EDWARD E. DASCHER

BY

*Edward E. Dascher*  
ATTORNEY

Nov. 2, 1965

E. E. DASCHER

3,215,558

**E. DASCHER** 3,2  
**METHOD OF COATING METAL FOILS WITH A POLYMERIZABLE**  
**RESINOUS COATING**

Filed Feb. 16, 1959

17 Sheets-Sheet 14



Nov. 2, 1965

E. E. DASCHER

3,215,558

METHOD OF COATING METAL FOILS WITH A POLYMERIZABLE  
RESINOUS COATING

Filed Feb. 16, 1959

17 Sheets-Sheet 15



EDWARD E. DASCHER

INVENTOR.

BY

*Edward Dascher*

ATTORNEY

Nov. 2, 1965

E. E. DASCHER

3,215,558

METHOD OF COATING METAL FOILS WITH A POLYMERIZABLE  
RESINOUS COATING

Filed Feb. 16, 1959

17 Sheets-Sheet 16



BY *Edward E. Dascher*

ATTORNEY

Nov. 2, 1965

E. E. DASCHER

3,215,558

METHOD OF COATING METAL FOILS WITH A POLYMERIZABLE  
RESINOUS COATING

Filed Feb. 16, 1959

17 Sheets-Sheet 17



EDWARD E. DASCHER  
INVENTOR.

BY *Alexander Duschner*

ATTORNEY

1

3,215,558

## METHOD OF COATING METAL FOILS WITH A POLYMERIZABLE RESINOUS COATING

Edward E. Dascher, 402 Garden Blvd., Garden City, N.Y.

Filed Feb. 16, 1959, Ser. No. 793,612

2 Claims. (Cl. 117—230)

This application is an improvement over and a continuation-in-part of applicant's pending application for patent on Electrically Conducting Adhesives and Foil Conductors filed on November 12, 1954, under Serial No. 468,391, now abandoned.

This invention relates generally to electrical conductors, but more specifically to the processing of electrically conducting metallic foils and dielectric coatings therefor, the apparatus used and the end products thereof.

The process, apparatus and resultant product of the invention constitute a novel departure from known processes, apparatus and products which involve (1) baking or curing of foil coatings for solvent evaporation or for modification of resinous or resin-forming ingredients; (2) laminations of metallic and non-metallic foils treated for bonding and/or for additional coatings and penetrants; (3) vapor deposition of metals on foil in vacuum; (4) and anodic oxidation of metals to serve as dielectrics.

Specifically, applicant simultaneously by a continuous and progressive process: (1) synthesizes, in successive stages of and by polymerization processes, a dielectric coating on one side of the metal foil, such synthesized coating including a formed modification of a polymer or copolymer, or a formed resinous polymer, or copolymer; (2) pressure molds the synthetic resultant uniformly, densely and by successive and fused deposition on the foil for dielectric gauge controlled development; and (3) anneals the metal foil component.

Thus, the invention lends itself to economic and high-speed production, gives the conductor longer life, more efficient performance and wider utilization.

Broadly, the invention provides an insulated electrical conductor for use in electric or electronic circuitry and in components of such circuitry, the said conductor having an electrically conducting metallic foil of selective gauge and a reinforcing dielectric plastic coating of selective gauge thermionically or molecularly bonded to the virgin foil metal and also mechanically bonded to the oxide thereof.

One of the objects of the invention is to effectuate and provide such a foil and coating with dimensional, textural and property uniformity and stability; with higher temperature operational characteristics involving less or no coolants; with no cold roll, creep or delamination characteristics in operation or during winding and stacking formation thereof; and with foil and coating characteristics of compatible and cooperative electrical, physical, chemical and thermal advantage.

Another object of the invention is to provide a conductor of the above nature and of selectable dimensions and values and embodying such electrical, thermal, physical and chemical characteristics as to allow economic, simplified and efficient fabrication therefrom of component parts or elements in electronic circuitry at the manufacturing or industrial site. Thus, the conductor is capable of delivery to the industrial site in continuous lengths pursuant to value specifications as in roll form and the fabricator engages in the required winding, stacking or other formable operation for the production of a component unit or other element in electronic circuitry. Thereafter, the formed unit is bonded by the fabricator by a simple reactivation operation of the dielectric for unit completion.

2

Another object of the invention is to provide a conductor of the above nature capable of use in miniature, sub-miniature and conventional electronic circuitry; capable of use as a fillable capillary and inflatable conducting tube for use in gauges, fuses, testing devices or other purposes as will appear; capable of reducing weight and space of components or elements formed of such conductor, and of uniformly and efficiently dissipating uniform heat development in each convolution or layer or lamination of the windings and stackings from such conductor to permit efficient and high voltage per mil of dielectric operation for longer hours, at higher temperatures, at substantially uniform performance and without or diminution of use of coolants.

Metallic foil heat developed in operation of the conductor of the invention as a wound or stacked component by reason of dielectric reflective, refractive and dispersive values is efficiently absorbed by the dielectric component for each convolution or lamination and is dissipated by continuous and immediate lateral emission and conduction to the component edges which are exposed for ambient temperature absorption. Such phenomena are attributable to the contacts between the dielectric, the oxide and the virgin foil, which involve molecular and mechanical integration and also to the homogeneous, dense and uniform gauge characteristics of the dielectric. There is further a complete absence of permeability, pockets and foreign material-containing areas between said contacts to eliminate resulting adverse effects.

A further object of the invention resides in the provision of a conductor having an annealed or oriented metallic foil component and a simultaneously oriented and pressure-compacted and uniform dielectric coating component at least on one side of the foil. The conductor, moreover, partakes of the physical and improved strength of the coating. Thus, conductors derived from metallic foil from about .005 down to about .000175 inch in gauge and dry coatings from .00025 down to .00001 inch in gauge have been formed, capable of utilization for fabrication. Of course, the conductor may have the uncoated side provided with a dielectric by subsequent operations and by any method.

Another feature of the invention resides in the improvement of the metallic foil component of the invented conductor as it comes from the rolling mill resulting from thermionic, pressure and annealing conditions.

Another feature of the invention resides in method, apparatus and product for forming either the conductor of the invention or any other type of conductor having a one sided dielectric coating into folded longitudinal edge form to control width and improve characteristics for component formation in circuitry.

Another feature of the invention resides in method, apparatus and product for forming the conductor of the invention or any other foil conductor having a dielectric on one side into capillary, fillable, inflatable and flexible tubular form to improve characteristics for component formation in circuitry and to serve other electrical functions.

These objects and other incidental ends and advantages of the invention will hereinafter appear in the progress of the disclosure and as pointed out in the appended claims.

Accompanying this specification are drawings showing various illustrative embodiments of the invention wherein:

FIGURE 1 is a view in perspective of the remote control panel for effecting operable conditions in the various and continuous sections of the reaction chamber or tower plant;

FIGURE 2 is a schematic view in perspective illustrating a preferred production assembly line for manufacture of a form of the conductor of the invention wherein:

shown a coating plant; the tower plant wherein heating, annealing, evaporation, combustion, synthetic product deposition under controlled temperature and pressure conditions, orientation and cooling take place; a slitting plant; an editing plant for imperfections; a folding plant for effecting one form of the invention; and an ultrasonic welding plant for the opposing edges of the folds;

FIGURE 3 is an enlarged sectional view diagrammatically showing molecular and physical bondage between the dielectric, the oxide and the virgin metal of the invented conductor and other characteristics;

FIGURE 4 shows an enlarged transverse sectional view of a flipped-over or folded edge formation of the invented conductor shown in FIGURE 3;

FIGURE 4a is a schematic overlap form of the conductor;

FIGURE 5 shows the conductor of FIGURE 4 in plural ply formation;

FIGURE 6 is an enlarged sectional view of a tubular form of the invented conductor;

FIGURE 7 shows the conductor of FIGURE 6 in plural ply formation;

FIGURE 8 is a view in elevation showing the conductor of FIGURE 6 in cylindrical form;

FIGURE 9 is a diagrammatic view taken transversely of results of a folding operation of one ply of metal foil with or without dielectric coating;

FIGURE 10 is a view similar to FIGURE 9 but with two plies of metal foil resulting from a folding operation with or without dielectric coating or other insulation;

FIGURE 11 is a similar view but with a plurality of plies of foil, plastic or other dielectric resulting from a folding operation;

FIGURE 12 is a fragmentary and diagrammatic view in perspective showing the metal foil as it comes from the rolling mill containing an oxide and protective mineral oil film plus a coating application for final synthesis of the dielectric coating;

FIGURE 13 is a fragmentary and diagrammatic view in perspective showing the specimen of FIGURE 12 after complete subjection to the vertical tower operation;

FIGURE 14 is a sectional view partly fragmentary showing a form of the coating plant, the entry feeds thereto the inlet feeds to the tower plant;

FIGURE 15 is a view in perspective partly broken away showing other details of the coating plant not shown in FIGURE 14;

FIGURE 16 is a view in perspective partly broken away showing details of structure for control of amount of coating application;

FIGURE 17 is a view in perspective of the plural tiers of the vertical tower plant and the external processing rollers and rewind of the processed foil conductor;

FIGURE 17a is a schematic view of FIGURE 17 exemplifying vertical operation and 17b horizontal operation;

FIGURE 18 is a fragmentary view in perspective of a detailed structure of a multiple flue associated with the tower plant for control of entry of selected values of cubic feet of air per minute thereto;

FIGURE 19 is a view in perspective showing preliminary arrangement prior to folding for aligning a plurality of laminations as seen in FIGURES 10 and 11;

FIGURE 20 is a diagrammatic view showing details of temperature and volumetrically controlled air supply to sections of the tower plant;

FIGURE 21 is a detailed view in perspective showing the top tier of the tower plant, structure for air introduction, heaters, and temperature reading instrumentation;

FIGURE 22 is a view in perspective of a bowed type of roller and the mounting therefor;

FIGURE 23 is a sectional view of FIGURE 22 across the plane 22—22 thereof;

FIGURE 24 is a sectional view of FIGURE 23 across the plane 24—24 thereof;

FIGURE 25 is a fragmentary perspective view partly broken away showing port and other details at the upper tower tier for discharge of products of combustion and other active fumes to a catalytic combustion chamber;

FIGURE 26 is a fragmentary perspective view at the top of the upper tower tier showing details of a top drum, controls therefor and dewrinkling rollers for the processed conductor;

FIGURE 27 is a diagrammatic and perspective view showing an air controlled dancing roller for the coated metal foil stock preliminary to feed into the tower plant;

FIGURE 28 is a view in perspective of a slitting plant for the completed and processed conductor;

FIGURE 29 is a view in perspective and partly diagrammatic showing editing or means for reading dielectric strength of coating on web after the slitting operation;

FIGURE 30 is a sectional view of FIGURE 29 across the plane 30—30 thereof;

FIGURE 31 is a view in perspective of apparatus for direct wind of the processed conductor adjacent the top of the tower plant.

*Basic considerations of invention—FIGURES 17a-17b*

For a broad comprehension of the invention before proceeding with a detailed description of apparatus, method and end product, brief reference is made at this portion of the specification to the treatment and mounting of the metallic foil stock coming from the rolling mill with the conventional oxide and mineral oil surface and to the manner and type of in situ synthetic formation and deposition of dielectric resin from the basic materials in the coating-all resulting in the fundamental structure shown in FIGURE 3.

The metallic foil stock whether aluminum or other non-magnetic and electrically conducting material including copper, is first subjected to a controlled thickness of coating on either side and then to movement under controlled velocity and controlled conditions of stretch or tension through a heating or reaction chamber 106 (see FIG. 17a) comprised of a plurality of communicating tiers 106a, 106b and 106c each having independent temperature as well as volumetric air-inlet systems, the latter being indicated by 109, 110 and 111 respectively. At the bottom of lowermost tier 106a are independently adjustable dampers 211 and 212 to control size of inlet 106a' for air inlet control and to admit coated foil or web 101a, while at the top of tier 106c and at roof portion 176 are independently adjustable dampers 185 to control exhaust of reaction gases and suspensions through the pair of exhaust conduits 186. The exhaust conduits communicate with an exhaust duct 113 having exhaust fan 112 and there are independently adjustable dampers 189 therebetween. On the top of roof 176 there is a closeable opening controlled by independently adjustable dampers 184 to form another adjustable air inlet 106c' for air downdraft for cooling and annealing purposes. Web 101a also emerges from inlet 106c'.

The air inlet systems 109, 110 and 111 for the respective tiers have direct entry (arrow indicated) on the uncoated side of the web through nipples 309a, 309b, and 309c while on the coated side of the web, entry is effected by branches 310a, 310b and 310c coming off chambers 308a, 308b and 308c.

The web 101a is under tension between lower roller 107 and top high and controlled constant torque drum 108 and is subjected in each of the tiers on both sides to various heats as afforded by resistance rods 115 or other heat producing means.

For making a dry coating of polyurethane of .00025 inch on aluminum foil of .0005 inch and of 12½ inches width from specified bath materials at a viscosity value of Zahn cup #4, twelve seconds, and wherein the tiers

are six feet high, eight by eighteen inches on the sides, with a metallic foil unwind speed of forty feet per minute, temperatures, air-intakes, exhaust and pressures must have specific values.

Thus, by again referring to FIGURE 17a, the updraft of air through bottom air inlet 106a' is about 150 c.f.m., the air entry for tier 106a is about 150 c.f.m., for tier 106b air entry is about 250 c.f.m. and for tier 106c, air entry is about 350 c.f.m. The downdraft through top air inlet 106c' is about 375 c.f.m., while the exhaust through duct 113 is about 350 c.f.m. Temperature in the tier 106a is about 500° F., in tier 106b about 750° F. and in tier 106c about 800°-900° F.

Pneumatic pressure on the uncoated side of web 101a is maintained at a higher value than on the coated side because of pressure conditions involved in the polymerization process and the depositions. This pressure differential may be accomplished in any suitable manner, but as seen in FIGURE 17a by branched feeds 310a, 310b and 310c to the tier sides facing the web coated side, by directional baffles 316c (seen in FIG. 18), and by differential manipulation of each of dampers 211-212, pair of dampers 185, pair of dampers 184, and pair of dampers 189.

The coating material of the bath in the example used and hereafter specified is adapted for in situ synthesis and successive and fused blow-molded depositions of high-polymeric macromolecular condensation and other compounds, and includes solids, liquids and active solvents therefor of different boiling points. Thus, in timed foil travel in chamber 106, the mill applied mineral oil 103 is substantially removed by fractional vaporization and the low boiling vaporized solvent is in a condition of polymerizable activity with the foil residue of the resin-forming materials. Then higher boiling solvents are vaporized to a condition of polymerizable activity and the foil residue itself is at least partly thrown into vapor pressure and suspended activity. All components and reactants are forced into close contact with web 101a by the air systems 109, 110 and 111 resulting in density of dispersion thereat and economy in minimizing loss through the exhausts.

Conditions in reaction chamber 106 caused by updraft through air inlet 106a', downdraft through air inlet 106c', air entry to the tiers through systems 109, 110 and 111, exhaust through duct 113, mobile vapor pressure equilibrium conditions of the bath ingredients and various temperatures, combustions near the rods 115 (highest temperature about 1500° F.) and pressures developed (Boyle's law) all contribute to not only resinification, modification or resin formation in situ but also to blow-molded successive and fused deposition of layers of high density, polymerized particle aggregates from the chamber contents. The pneumatic pressures and directions thereof within the chamber prevent the foil coating from free run-down and further serve as a brush type of molding for uniform distribution. The pressure of the reaction chamber 106 on the uncoated side necessarily exceeds that on the opposite side to serve as cushioning for the delicate foil gauges against the pressure effects from the coated side. If this type of posturing were not so, the foil, owing to its perforated and striated nature as it comes from the mill, would become perforated and adhesively wrinkled with resultant shear, strain and tearing.

In the reaction chamber 106, the metal foil component is elongated at about 450° C. whereby the stock variations in gauge is reduced, the texture is made uniform, free of gaseous, solid and fluid impurities and spatial imperfections, and is also annealed. Moreover and as seen in FIGURE 3, the conditions described and as indicated cause a thermionic type of bondage of the underlying resinous layers 138 to the virgin metal 137 (latter being excited to electronic emission) and through the interstices of the oxide of the foil as at 141 while also being mechan-

ically and pressure bonded to the oxide 139 as at 140 disposed over the virgin metal.

Fused redepositions under blow pressure effect uniformity and density of dielectric gauge and elimination of pockets, trappings and lamination facings, the latter being existent in other methods of plural coatings by redips or the like.

Moreover, the formed dielectric coating is subject to simultaneous annealing or orientation with the metal foil component by slow cooling at the upper part of the tower owing to the downdraft through inlet 106c'. As a result, the dielectric texture has improved thermal and dielectric characteristics and transfers to the captive annealed foil its own higher values of tensile strength, impact resistance, and resistance to shear and pressure. Furthermore, the thermionic, or molecular type of bonding described, eliminates cold roll or creep due to varying conditions as etching and high temperature effects and eliminates deformation in stacking due to developed inside pressures.

Electrolytic factors exist in reaction chamber 106. Water from the condensation reactions is present in vapor form and other ionized groups are present. To prevent oxidation of the metallic foil, the pH value should be on alkaline side such as pH 8 at the exhaust area. The conductor on emerging from the chamber is at about pH 7, while the pH of the coating bath is pH 9-pH 11.

By reason of the aforementioned processing and treatment, there results a conductor (see FIG. 3) of which the annealed captive foil component 137 has better and more uniform electrical, thermal, flexible, forming, shape-conforming, foldable, windable and stackable characteristics than the foil stock 100 itself; the oriented dielectric component 138 is dense, uniform in gauge and texture, is not subject to cold roll or creep in production techniques required by reason of molecular and physical anchorage to the annealed metal component and has folding, creasing, winding, stacking and shape-conforming characteristics.

The conductor comprised of the foil and dielectric coating as described when in tightly wound or stacked formation for resistance, capacity or other electrical function is capable of being bonded by the fabricator thermally as by induction after stacking or winding, or by the use of a solvent during stacking to integrate the unit. Even when the dielectric coating is of thermoset resin, nevertheless, it is controlled in the chamber for an intermediate stage of polymerization and is thermoplastic, but induction heating by the fabricator completes polymerization to infusibility.

The conductor after slitting operation as seen in FIGURE 28 and to be described is capable of use in strip form and also in longitudinally-edged folded condition as indicated by numerals 127 and 127a in FIGURES 4 and 4a respectively. Such folding when the conductor is used for winding or stacking purposes eliminates the necessity of etching for uniform width, increases tensile strength and reduces possibility of shorts of the convolutions or plies as seen in FIGURES 5 and 7. Moreover, when the opposing edges are integrated such as at the butt 142 by ultrasonic welding as indicated by 142' in FIGURE 6 and shown in resultant forms 144 and 129 in FIGURES 7 and 8 respectively, the conductor may be wound or used independently as a capillary. Such capillary is fillable and inflatable for electronic circuitry function either as a conductor, gauge, trip, fuse, capillary tube systems as in refrigeration, etc.

#### Bath ingredients

The bath ingredients 105 in tank 208b is applied to foil 100 as it comes from the mill and on either side. This is done continuously by doctor roller 104 on either side of the foil to form travelling web 101a which proceeds through the reaction chamber 106 as best seen in FIGURE 14. The bath includes materials for ultimate syn-

thesis into high polymeric and copolymeric or high polymer or copolymer modifications by condensation and other processes. The polymerization reactions are macromolecular but addition types are also contemplated.

Depending upon operational temperature requirements, synthesized coating resins are of both thermosetting or thermoplastic varieties and include:

- (1) Vinyl polymers including polyvinyl chloride
- (2) Phenolics and modified phenolics
- (3) Polyesters including alkyds and modifications thereof by silicones
- (4) Cellulosics including cellulose acetate, cellulose acetate butyrate and ethyl cellulose
- (5) Epoxies
- (6) Polyurethanes.

The basic materials found satisfactory in coating bath 105 for development of the dielectric coating 138 and involving a polyester modification of an alkyl (three-dimensional polyester) in the example used herein for a .00025 inch dry coating on a .0005 inch aluminum foil is substantially as follows:

40% solvent contents of which toluene comprises 10 parts; xylol comprises 25 parts; and methyl ethyl ketone (for a mineral oil removal on mill foil) comprises 5 parts; and

60% soluble contents of which diallyl phthalate polyester already modified by triallyl cyanurate comprises 40 parts; cresylic acid comprises 14 parts; glycol comprises 5 parts; and polyhydric phenol (inhibitor) and dialkyl aromatic amines (catalyst to promote cross linkage reactions in tier 106c) together comprise 1 part.

The modified polyester dry coating 138 affords the characteristics herein stressed including flexibility, heat-stability, excellent abrasive resistance, formability, heat permeability, constant dielectric strength, thermionic bonding with virgin metal and favorable refractive, reflective and dispersive heat wave values exemplified in FIGURE 3.

Of the list of six synthesized resins heretofore mentioned, numbers "2," "3," and "6" are substantially included in the above formulation; but the balance of the said list would involve variations in ingredients of the bath 105, which, however, would be subject to the same tower and other environmental conditions. Other ingredients for silicone formation may be added to increase higher temperature tolerance for a polyurethane formation, while various other catalysts and regulators may also be used. The coating composition is controlled for viscosity for required conditions of foil application and synthetic resin deposition as by meter 222 in FIGURE 14.

The dielectric coating as synthesized herein (resulting in condensation polymerization from ingredients given) is formed under conditions of relatively low temperatures and pressures. The use of active solvents in the synthesis involved do not involve high heats of reaction and temperatures; they are controllable since the solvent acts as a heat transfer medium and causes agitation during polymerization. Final products of intermediate polymerization stage are formed for thermosetting coatings for thermoplastic condition and are rendered thermosetting by the fabricator in the final bonding by induction operation or otherwise.

#### *Efficiency and economy of conductor*

With the bath ingredients used and for a dry dielectric coating of .0025 inch and an aluminum foil of .0005 inch on a conductor of the invention such as 127 (FIGURE 4), the conductor under test in wound form and before integration by the fabricator withstood 240 volts per  $\frac{1}{4}$  mil of dielectric and after integration by the fabricator withstood 640 volts per  $\frac{1}{4}$  mil of dielectric with operating temperatures of 100,000 hours at plus 155° C. and 1000 hours at 270° C. Thus, the conductor is capable of continuous and efficient operation at elevated temperatures and for high voltage owing to immediate

and uniform absorption of the generated foil heat by the dielectric and immediate, efficient and continuous lateral transfer of the heat to the lower and ambient temperature at the conductor edges. This is illustrated in FIGURE 3 by thermal arrow lines and also by heat conducting channels 141 at the interstices of the oxide crystals 139. The original oxide layer or barrier 102 is broken and prevents heat accumulation.

For economy of production of the conductor of .0005 inch aluminum foil and .00025 inch polyurethane dry coating, three quarts of the bath make about 500 square feet of foil under these approximate conditions of operation (see FIG. 17a):

- 15 (1) Web feed speed (at pinch roller 208a) is 40 feet per minute.
- (2) Web width is 12½ inches.
- (3) Tier cross-sectional dimensions are 8 by 18 inches.
- (4) Air inlet at 106a' is 150 c.f.m.
- 20 (5) Tier 106a temperature is at about 500° F., and air inlet through 109 is 150 c.f.m.
- (6) Tier 106b temperature is at about 750° F., and air inlet through 110 is 250 c.f.m.
- (7) Tier 106c temperature is between 800°-900° F., and air inlet through 111 is 350 c.f.m.
- 25 (8) Downdraft c.f.m. through inlet 106c' is about 375 for annealing.
- (9) Exhaust draft at 113 is about 350 c.f.m.

30 Of course, above nine conditions or values are all variables, specific values depending upon requirements of group of dielectric, gauges, and specific metallic foils. Variations in chamber structure and dimensions will also affect values.

#### *Tier activities: 106a*

Under the example given for production of .00025 inch dry dielectric of polyurethane on .0005 inch aluminum foil as it comes from the mill and when reaction chamber 106 is in vertical position (different temperatures, air pressures and other conditions apply when disposed off vertical as in FIGURE 17b), the coated stock 101 under tension between bottom roller 107 and upper drum 108 passes through tier 106a where volatilizing of mineral oil and one or more of the solvents takes place. The coating is comprised of many fractionally distillable components to which the timing of and exposure to respective tier temperatures and pneumatic pressures are controlled and geared.

45 In the lowermost tier 106a, most of the degreasing takes place by fractional evaporation of the mineral oil and of one or more of the solvents of lower boiling points. Air controls for temperature and pressure requirements and for reaction flow in the reaction chamber 106 include as stated the bottom inlet 106a' (FIG. 14), directionally, 50 volumetrically and temperature controlled pairs of air inlet systems 109, 110 and 111 for tiers 106a, 106b and 106c respectively (FIG. 21) and exhaust 113; top air inlet 106c' for downdraft being provided for controllably applying an air coolant for annealing and orienting purposes at the top of the reaction chamber (FIG. 25).

55 Updraft in the reaction chamber is facilitated by exhaust fan 112 of variable capacity outside of and adjacent the uppermost tier 106c and leading to the catalytic chamber 114 (FIG. 20). This updraft by way of duct 113 removes unreacted fumes, vapors, gases and suspensions.

60 Temperature in tier 106a is maintained at about 500° F. at the junction with tier 106b. Controlled degree of heat within the several tiers in addition to that afforded by heats of reaction and combustion is furnished by electrical resistance rods such as 115 seen in FIGURE 21. Such rods are disposed throughout the reaction chamber, on both sides of the web 101a, suitably sheathed, the emission temperature of the rods on the coated side under 65 the conditions herein being greater than on the uncoated

side. Maximum sheath temperature in the tower is about 1500° F. Other heating means may be introduced.

Within tier 106a, free run-off of the web coating due to gravitational forces is opposed by: the adjacent updraft pressure from air inlet 106a'; opposing pressures from air inlet system 109; the rising of vapors adjacent the coated web side from evaporation of the mineral oil, and the low boiling solvents, all while the web is postured both under controlled tension between rollers 107 and 108 and by said opposing pressures, the latter maintaining the reagents close to the web for increasing dispersion density, and resultant efficiency and economy of operation. Thus, an air brush and blow pressure type of distribution is provided for the coating within tier 106a wherein combustions or small explosive reactions take place adjacent rods 115 of both the solvent and mineral oil vapor. Annealing of metallic foil 100 also commences in tier 106a owing to heating and stretching conditions of the foil. Controls such as by dampers for air inlets and exhaust and for temperatures will be detailed hereafter.

#### Tier 106b

As the web approaches tier 106b, the succeeding reaction chamber, reactions other than those that took place in tier 106a take shape. Although velocity of movement to chamber inlet 106 is about 40 feet per minute as stated, this speed depends upon varying conditions including metallic foil thickness, coating or resin group, thickness of coating material, temperature conditions, required dry dielectric deposition, thermal bonding of convolutions after dielectric deposit, and also other factors. Empirical formulae are establishable to modify all values set forth in this specification to accomplish the same results.

The temperature in tier 106b at the junction with tier 106a is at about 750° F. and the coating is in a soft gel state, traces of unevaporated mineral oil and low boiling solvents being now readily evaporated. Air, under volumetric, directional (FIG. 18, 316c') and temperature control (FIG. 20, 307) enters through the air inlet system 110 on both sides of the web for support and posturing of the web during its movement along the tier and to maintain dispersion density adjacent the web. Solvents of higher boiling points evaporate in tier 106b carrying the unexhausted mineral vapor in solution upwardly to prevent possible contaminating mineral oil redeposition on the coating due to air pressure from inlet system 110 toward the coated web side. Sparking and ignition of freely suspended constituents also take place adjacent the heater rods in tier 106b. Vapors, suspensions and other floating particles rise into tier 106c for possible reaction therein and the excess is sucked out through exhaust duct 113 to the catalytic chamber 114 for complete combustion.

#### Tier 106c

The web coating at the junction of tiers 106b and 106c whereat the temperature is between 800-900° F. is now in a uniform, non-flowing and reactable condition for final, successive and fused dielectric deposition. The web assumes a moderate draping, becoming more pronounced as it is forced or passes closer to the heating rods 115 by tier activity. Elongation is taking place and slack is opposed by dancing roller 120 (FIG. 27).

Annealing of foil 100 is now under way, the foil being in a soft condition and exhibiting the physical characteristics of the coating rather than the metal thus preventing foil strains and shear leading to tear. Air entry through air inlet system 111 contributes to the pressures and currents within tier 106c, pneumatic pressure on the uncoated side of the web being greater than on the other as heretofore stated to serve as a yieldable cushion for vapor pressure and successive deposition, while the down-draft from top air coolant inlet 106c' is at work to anneal the foil, to massage down the coating within tolerances and to orient same. The air updraft is finalized and

channels the movement of unuseable or excess toxic, gaseous and suspended material into exhaust duct 113 for incineration (or for reclamation) in catalytic chamber 114.

5 At the time of traverse of web 101a through tier 106c, the coating has been substantially freed of solvent and other original constituents and constituents of reaction of the coating material, leaving a bonded and plastic-conditioned residue in vapor pressure equilibrium condition thereon. Under pressure, temperature and reaction conditions commencing at the upper part of tier 106b, the bonding of the undermost constituents of such residue to the foil and oxide is as heretofore stated apparently thermionic and also definitely mechanical.

10 Thus, during traverse in tier 106c, the residual foil coating is in activated condition, the underlayers being thermionically or molecularly bonded to the virgin metal through the oxide interstices 141 (rearranged by the annealing process) while the outer layers in mobile vapor pressure condition of equilibrium successively build

15 up with the tier contents under the conditions therein fused upon fused layers of synthesized polymers, copolymers and modifications thereof. Opposing air pressures from system 111 effects uniform molding of the depositions fusing layer on layer, causes dense deposits and eliminates pockets, removes traces of all impurities and other adverse conditions.

20 Now, a selectively and controlled degree of polymerization, orientation and annealing takes place during ascent in tier 106c wherein air of selective temperature is drawn downwardly from top air inlet 106c' (FIG. 25) through dampers 184 for curing and final annealing of the conductor.

25 The coating bath ingredients 105 may have color pigments including the aniline dyes for giving the final dielectric deposit coding colors such as green, red, blue, black etc. to follow similar color codings found in wire systems and to serve as polymerizable ingredients.

#### Web processing after exit from reaction chamber

30 The conductor so formed and constituting the annealed foil component 137 and the oriented dielectric deposit 138 is now behaving as a resinous sheet in full drape with a captive and annealed metallic foil as same leaves the roof 176 of tier 106c through roof opening 179 as seen in FIGURE 26. This drape is immediately straightened out by an underwrap of the web with a first bowed roller 326 and an overwrap with a succeeding roller 327. To prevent adding more strain to the entire web at this area, a wrinkle is imposed by a succeeding underwrap with bowed roller 328 and the imposed drape is straightened to a depth of many feet by the successive passage over drum 108 by a reason of the high torque and circumference thereof. Drum 108 also uniformly cools the emerging web 101a in its traverse thereover and frictionally burnishes the uncoated side of film layers due to deposition of migrating vapors. The web proceeds downwardly and makes an underwrap with alternate and opposite bowed rollers 328a and 326a and an overwrap with intermediate roller 327a. Drum 108 and rollers 326-328, and 326a-328a are all mounted in top framework 195 as seen in FIGURE 26.

35 In this manner, lateral strain, shift and shearing is prevented. The web as it continues its passage over other processing rollers is now a smooth continuous one.

40 As seen in FIGURE 17, other suitable controlling means for proper tension, strain reducing and other tempering and processing functions are provided and mounted on a side of the reaction chamber 106 before rewinding of the completed conductor takes place on bottom rewind roller 121, including roller 116a, bowed rollers 116-118, roller 117 intermediate thereto and additional processing rollers 121a-121j inclusive. All the rollers 45 are statically and dynamically controlled and the fric-

tional passage of the processed web over such rollers and especially over top drum 108 as above stated which has torque control 329 for tension requirements, causes a removal of any deposited film on the uncoated side. Such film is very light and is caused as stated by eddy currents of the vapors and suspensions taking place in the reaction chamber 106. There is no bondage of such film on the uncoated side of the web due to absence of conditions obtaining in the chamber opposite the uncoated side.

*Modification of web processing after exit from reaction chamber*

A modification of roller processing as by bypassing rollers of FIGURES 17 and 26 is shown in FIGURE 31 for accommodation of metallic foils of the lighter and heavier gauges.

The rewinding of conductors of lighter gauge metallic foil on bridge 800 adjacent chamber roof 176 as distinguished from rewind 121 at the lower end of the roller assembly (FIG. 17) is to assure proper mechanical conditioning without further roller or mechanically-hardening such lighter gauges. Such a precaution is to prevent possible rupture by needless additional hardening of lighter gauges.

Similarly, in the case of conductors of heavier gauge metallic foil, there is no need to reharden or retemper following the annealing and polymerization process effected in the chamber 106. Moreover, the effects of the dead weight of the web are eliminated by roller assembly shown in the modification of FIGURE 31.

In FIGURE 31, a framework 801 extends from the floor of bridge 800, said framework carrying the rewind shaft 802 driven by variable speed and torque motor 803 through reducer 804 connected to electric clutch 805 by chain 806. An instrument panel has alternating current conversion controls 807 for motor operation and alternating current conversion controls 808 for electric clutch 805. Numeral 809 indicates a switch for motor 803.

Thus, web 101a as it proceeds from roof 176 to rewind shaft 802 proceeds under bowed roller 326, over roller 327 and 327a, and on the downward run passes under bowed roller 326a under roller 810 for rewind on shaft 802.

*Conductor slitting and editing*

Further procedures affecting the completed conductor may proceed. As seen in FIGURE 28, the treated foil from the rewind roller is dimensionally slit from the dielectric side by a compound and controllably operated slitting mechanism generally indicated by numeral 122 for rewind on compound rewind shaft 123. There is a variable speed and torque controlled motor 501, a constant torque control 502 connected to rewind shaft 123, cutters in the form of adjustably spaced razors 503 for slitting the stock from the dielectric side. Controlled pneumatic devices for constant torque control are used for operating the yoke frame on one arm of which is mounted the shaft 503a for razors 503 and on the other arm of which is mounted pressure shaft 503b for the winds on shaft 123. Thus, the pneumatic devices each have a chamber 504 having piston 503 therein and connected to the end of yoke arm 507. Air from a compressor is introduced into each of chambers 504; the latter have controls for maintaining or changing piston pressure. The base of the yoke is connected for pivotal movement on bearing blocks 509. Thus, stock 101a passes under roller 508 and shaft 503a for penetration and cutting by razors 503 and for rewind on shaft 123.

A novel editing system for the conductor strips is shown in FIGURES 29-30 wherein 601 is a combination oscilloscope voltmeter to read dielectric strength of coating. 602 and 603 represent spaced rotatably and suitably mounted pinch probes 602 and 603 cooperating with the

5

10

15

20

25

30

35

40

45

50

55

60

65

70

75

change-of-direction and free-rolling rollers 605. As slit and coated conductors 604 pass between the rollers, the probes make contact with the dielectric side to determine condition thereof and for indication on the instrument 601.

From any of the rolls shown in FIGURE 28, the conductor may proceed to a folding process and apparatus indicated in FIGURE 19 to arrive at the products 127 and 127a as shown in FIGURE 4 and 4a and the products 146 and 147 seen in FIGURES 10 and 11. After folding, the conductor may proceed to a welding process and apparatus to arrive at the products 129 shown in FIGURES 6 and 8.

*Controls and continuous coating, slitting, editing, folding and welding system*

FIGURE 1 shows the remote control panel for the coating system and will be discussed hereinafter following more detailed fill-in of structure involved.

A continuous system of coating, slitting, editing, folding and welding is schematically shown in FIGURE 2 and briefly involves a continuous, substantially enclosed and consecutively operative coating, slitting, editing, folding and welding system to arrive at a tubular type of conductor such as 129 shown in the forms of FIGURES 6, 7 and 8.

In FIGURE 2, foil 100 from unwind roller 100a passes through a horizontally disposed and encased coating plant 130, the coated web or foil 101a then proceeds up reaction tower 131, down and externally of said tower into a horizontally disposed and encased slitting, editing, folding and ultrasonic welding plants 132, 133, 134, 135 respectively for ultimate rewind on roller 136. Details of editing, folding and ultrasonic welding will appear hereinafter.

*Additional apparatus details for coating plant*

Coating plant details are shown in FIGURES 14-16 inclusive.

Thus a constant torque and variable speed motor 201 (FIG. 14) through suitable transmission drives coating head roller 202 adjustably supported within bath 105 of tank 208b for transfer of a controlled thickness of liquid coating material to doctor roller 104. Rollers 204 and 205 are pressure rollers on each side of doctor roller 104 which in conjunction with dancing roller 120 maintains the coated foil or web 101a under tension for entry into reaction chamber 106 by a change of direction roller 107.

Roller 208 is the final control feed roller prior to entry over bath tank 208b and is associated with a vertically controlled and adjustable pinch roller 208a synchronized by gearing (not shown) with the gearing 237 of coating head roller 202 for similar speed; and is also electrically connected (not shown) to the rewind shaft 121 for signalling or indication of required tensioning. Pinch roller 208a controls the speed of entry into the system of the foil 100 and squeezes out required feed footage per minute. An indicator attached to pinch roller 108a (not shown) may thus indicate the speed of web inlet travel.

Coating tank 208b (FIG. 14) has an exit port 214 for overflow to a reserve tank 216 forming part of a circulatory system comprising pump 215 which feeds tank 208b through port 217 above. A viscosity meter 222 is between pump 215 and port 217 and a filter screen unit 219 is between tank 216 and pump 215. An entry 218 is provided for replenishing tank 216.

In FIGURE 15 a transparent enclosure 221a is provided for protecting the coating plant, the enclosure being capable of removal in sections.

As seen in FIGURE 15, the rolling mill stock of foil 100 is on unwind roller 100a provided with an electric torque clutch 222, while 224 and 225 are free bearing rollers dynamically and statically balanced for keeping accurate and specified tension and for taking out wrinkles from foil 100. Numerals 227, 228 and 229 represent special pillow blocks with adjustment for lateral and vertical movement.

cal traverse of rollers 224, 225 and 208. A control 230 for coating head 202 is provided and there is a separate power switch 231 for a torque control brake. Control or dial 230 is connected to one of the ears 202a of coating head roller 202 which is adjustable for depth of penetration into bath ingredients 105 as shown in FIGURE 16. Ears 202a rest on a pair of pivoted bars 235. Dial 230 is connected to a shaft 232 carrying a pair of fixed and spaced cams 233 each of which is adapted to ride on lower cam faces 234 of the arms 235.

Power for transmission to the coating head roller 202, for the doctor roller 104, and pressure roller 205 comes from transmission shaft 236 which is connected to motor 201. By adjusting dial 230, the coating head roller 202 as seen in FIGURE 16 can be controlled for depth of deposition and for transfer to doctor roller 104.

In FIGURE 14 is shown the entry of coated web 101a into reaction chamber 106 through the common entry port 106a'. The said port is formed as an example by a pair of adjustable dampers 211 and 212 each having controls 209 and 210 respectively for c.f.m. adjustment. Controls are micro-adjustable.

In FIGURE 25 is shown adjustable structure for down-draft air entry port 106c', and adjustable structure for exhaust control through conduit 113 leading to catalytic chamber 114 through a controlled exhaust fan 112. Thus chamber 106 at top has a roof structure 176 having a flange 177 at the open bottom for connection with the top tier flange 175 (FIG. 21). 178 is the top wall of the roof, 179 is an aperture therein, 180 and 181 are the side walls of the roof each having upper and lower slits 182 and 183. Upper slits 182 are for controlled horizontal movement of baffles or dampers 184 to control opening in roof aperture 179 for forming entry port 106c'. The lower slits 183 are for a pair of dampers 185 to control exhaust conduits 186 disposed on each web side for varying c.f.m. by covering bottom openings 188. Roof end wall 187 carries the exhaust duct 113 into which exhaust conduits 185 communicate, extent of communication being controlled by vertical baffles 189 penetrating roof top wall 178.

Dampers 184 are independently controlled by micro-adjustment controls 184a and indicators 192; dampers 185 by micro-adjustment controls 190 and indicators 191; dampers 189 by micro-adjustment controls 193 and indicators 194. All of said controls may be remotely controlled.

In FIGURE 20 is shown an air blower 206 communicating with a heater such as gas heater 307 for controlled distribution to pairs of opposite reaction chamber flue chambers 304a, 304b and 304c. From heater 307 the air branches out into couplings 308a, 308b and 308c (see also FIG. 21); thereafter branching off for entry into the respective flue chambers 304a, 304b and 304c by means of nipples and conduits as seen in FIGS. 20 and 21. For tiers 106a, and 106b the nipples 309a and 309b are shown in FIG. 17a, but for tier 106c, nipple 309c is seen in FIGURE 21. The conduits shown are indicated by 310a for tier 106a, 310b for tier 106b and 310c for tier 106c.

As seen in FIGURES 18 and 20, there is associated with each flue chamber a volume and directional control for air entry into the tiers of tower 106 and on both sides of web 101a. Although control shown in detail in FIGURES 18 and 20 is applied to the chambers 304c in tier 106c, the structure is the same for the other two chambers 304a and 304b in tiers 106a and 106b.

Thus from FIGURE 18, 311c is a control associated by gearing 312c with an arm 313c of a damper plate 314c rideable over openings 315c in the side wall of the reaction chamber tier 106c. Damper plate 314c also has openings 316c registerable with openings 315c for changing orifice size. Damper plate 314c is provided with a dial 317c associated with a calibrated box 318c to indicate damper control. The damper plate 314c is also pro-

vided with controllable directional baffles indicated by numeral 316c' for entry direction into the tiers and for c.f.m. volumetric control. All mentioned controls in this paragraph may be remotely mounted.

Again referring to FIGURE 21, 319c represents a dual thermocouple for reading air temperature in tier 106c and skin temperature of web 101a therein, and 320c for reading rod sheath temperature in tier 106c. Similar temperature reading thermocouples are associated with each of the two other tiers 106a and 106b. Also in connection with FIG. 17, 301 represents the bottom rewind variable speed and constant torque motor, 302 is the drive connected therewith. 303 is an electric eye suitably connected for lateral displacement of rewind shaft 121 (connection not shown) for evenly winding the processed and completed conductor.

In FIGURE 31, electric eye 811, shown coupled to a driving shaft of rewind roller 802 on bridge 800 controls lateral displacement thereof for even rewind.

FIGURE 27 shows the mounting for dancing roller 120 as by means of self-adjusting brackets 330 and 331 provided with air cylinders 332 and 333 respectively, the cylinders carrying respective pistons 334 and 335 for control of tension by the air dancing roller 120. Such self-adjustment maintains the coated stock 101a under required tension during annealing and stretching orientation in reaction chamber 106. Numeral 336 indicates a series of bypass valves and controls to maintain constant air pressure in the cylinders.

The anti-wrinkling and adjustable bow rollers used herein are exemplified in FIGURES 22-24. Thus roller 116 is mounted on self-adjusting bearing blocks 321 which engage projecting ears 321a of the bowed core 325. Micro-adjustment pins 322 adjust the roller for horizontal location, and axial multiple bearings 323 are interposed between the core 325 and the rubber (silicone or other suitable material capable of contacting coating of web 101a) sleeve 324. The bow is curved in the direction of traverse of web 101a as seen in the drawings.

#### Control panel

The control panel generally indicated by numeral 400 has a lower and upper portion 401 and 402. In the lower panel portion are temperature indicators of heat conditions in the various chamber tiers.

For tier 106a, 403a is the indicator for average temperature therein while 404a is for air-intake temperature of system 109, 405a is for web temperature from uncoated side and 406a is for rod 115 temperature. Indications are also present for normal operating temperatures in such areas.

For tier 106b, 403b is the indicator for average temperatures therein, 404b for air-intake temperature of system 110, 405b for web temperature from the uncoated side and 406b is for rod 115 temperature. Indications are also present for normal operating temperatures in such areas.

For tier 106c, 403c is the indicator for average temperature therein, 404c for air-intake temperature of system 111, 405c for web temperature from the uncoated side and 406c is for rod 115 temperature. Indications are also present for normal operating temperatures in such areas.

On one side of panel portion 402 are controls for the coating system. Numeral 407 generally indicates the controls for the variable speed and constant torque motor 329 driving drum 108 (FIG. 26), 408 generally indicates the controls for the rewind shaft 802 on bridge 800 (FIG. 39) and for rewind shaft 121 at the bottom of the chamber 106 (FIG. 17). 409 generally indicates controls for unwind shaft 100a (FIG. 15) and particularly the electric constant torque control clutch 222. 410 generally indicates the controls for applying selectively gauged coatings to doctor roller 104 (FIG. 16). Other controls and readings may appear (not shown) in con-

nection with maintenance or change of tension mechanisms throughout the system from unwind shaft 100a to rewind shaft 121.

On the other side of upper control panel portion 402 are the indicators for conditions in the catalytic chamber 114 as 411 for entry temperature of exhaust gases and 412 for discharge temperature after combustion. Entry temperature under aforeoutlined physical conditions is about 600° F. and discharge temperature is about 1050° F. Indicators 411 and 412 have set needles for maximum permissible temperatures. When indicator 411 shows a temperature beyond the setting, temperatures in the chamber 106 are too high and therefore require adjustment by checking c.f.m. and other temperature conditions. When indicator 412 shows a temperature beyond the setting, this is an indication that more air is required in the catalytic combustion chamber.

Indicators 413, 414 and 415 are lights energized by thermocouples in the catalyst of the catalytic chamber and indicates normal and abnormal gas and suspension mixes coming from the exhaust of reaction chamber 106. Lighting up of indicator 413 indicates a normal mix which ignites properly in the catalytic chamber; lighting up of indicator 414 means below normal temperature operation, and too much air is present; lighting up of indicator 415 means above normal temperature operation and excess solvent vapor is present.

Numerical 416 is an audible signal reflecting the condition of light 415, and 417 is another audible signal reflecting the condition of light 414. Switch 418 is the start and stop control for exhaust fan 112 which also serves as a blower for the catalytic chamber 114; 419 is a jet flame off-button and 420 is the jet ignition button.

Although not shown in the drawings and on control panel 400, c.f.m. indicators are provided at all air-intake and gas exhaust ports (see FIG. 17a) and panel remote readings therefrom may be provided. Moreover, c.f.m., temperature and other controls for normal operation as heretofore described may also be operated from the control panel 400, although not shown.

#### Folding

In connection with the arrangement and folding of plural conductors 146 and 147 (FIGS. 10 and 11) a system such as shown in FIGURE 19 is resorted to and includes a pair of upper and spaced statically and dynamically controlled unwind rollers or shafts 148, 149, and a pair of lower and spaced unwind rollers or shafts 150 and 151 also statically and dynamically balanced. Each of said rollers carries a coated or uncoated metallic foil, or a non-metallic foil for insulation between uncoated and naked metallic foils to arrive at combinations of metal foils insulated from each other and of different elements or alloys for electronic circuitry purposes, or as flexible and shape conforming cables. All the foils as shown are of the same width and are indicated by numerals 152, 153, 154 and 155.

Upper rollers 148, 149 feed strips 152 and 153 in contacting relationship while the lower rollers 150 and 151 also feed strips 154 and 155 in contacting relationship. Strips 152-153 and 154-155 join between pinch rollers 156 and 157 and proceed in contacting relationship through an aligning and compressing tubular member 158, then through another set of pinch rollers 159-160 and then into a folding mechanism for frictional integration and permissive separation at the terminal ends for connection to suitable conductors.

In the unwinding of rollers or shafts 148-149 and 150-151, variable speed and constant torque control motors 161-162 are provided each also having brakes and torques controlled transmissions 163 and 164 respectively.

The gear train for shafts 148 and 149 is indicated generally by 165 and that for shafts 150 and 151 is indicated by numeral 166.

#### Specific structural features

The fundamental conductor structure as seen in FIGURE 3 and being one of the subjects of the invention is comprised of annealed foil 137 and on the previously coated side is molecularly bonded as at 141 to the cured or partially cured dielectric and synthesized deposition 138 through the interstices of the foil oxide 139, while the latter, owing to its grooved, packed and bundle-like texture as schematically shown at 139, is also anchored mechanically to the synthesized deposition 138 as at 140. As shown by substantially vertical and horizontal thermal lines, heat from annealed foil 137 and developed in electrical operation is uniformly absorbed by the superposing synthesized dielectric resinous deposition 138 and emitted substantially laterally for escape through the edges of the conductor. Thus, the conductor edges serve as cooling fins, and there is no oxide barrier for localization or retention of heat in foil 137 developed under operating conditions since the heat constantly passes through the oxide interstices at 141 where there is the molecular bond between the synthesized dielectric resinous deposition 138 and the annealed metallic foil 137. It is here to be noted that no bonding agent under the invention herein is required between the coating and the foil.

Mechanically flipped-over or folded species of the conductor of FIGURE 3 are shown in FIGURES 4 and 4a and are indicated generally by numeral 127 and 127a. As heretofore mentioned, effective area is maintained and superior voltage rating, capacity, life and operation near the dielectric charring temperature results. Of course these attributes are also applicable to the unfolded species or the conductor of FIGURE 3 wherein by virtue of structure all species are resistant to fracture or rupture. Moreover, the conductor structure by virtue of its process of manufacture as described has no pockets, no foreign occlusions, has uniform texture, homogeneity and gauge and is not subject to cold flow during folding and pressure application. There is no local heating, no power losses and has uniform breakdown strength and zero shorts per square yard.

The flipped-over species 127 as shown in FIGURE 4 has the opposing edges thereof substantially in the form of a butt joint, the distance 142 therebetween being minimal and controllable. Numerical 127a indicates the overlapped species or folded foil. Tensile strength of such a flipped-over conductor and overlap type is increased for tight winding and stacking. As seen in FIGURE 5, coil 143 has the edges of all convolutions in alignment (applicable to species 127a) thereby eliminating necessity for etching; the convolutions are amply protected against short-circuiting and the width of the conductor is controllable to precision in the folding operation. Flipped-over conductors 127 and 127a may be stacked or festooned for different types of winding.

When the butt space 142 is closed, as by ultrasonic welding, a capillary type of conductor results as indicated generally by numeral 129, said conductor being indicated in blown condition in FIGURE 8 and in flat and wound condition as indicated by numeral 144 in FIGURE 7.

The conductors 127, 127a and 129 (FIGS. 4 and 6) after winding and stacking operations by the fabricator are then integrated by induction as a subsequent fabricator operation as heretofore stated for completion. Or, a solvent may be used during the winding and stacking for integration purposes. Following such integration, no other operation is necessary such as addition of another insulating coating, impregnating under vacuum, potting, etc. Additions, however, may be made.

The conductors described are applicable to production of electronic components including transformers, traveling wave tubes, magnet wave coils, capacitors, condensers, solenoids, horn-buttons, alternator rotor coils and potentiometers (latter use as by drape or festoon stacking).

Results of flip-over or overlap of metallic and other

foils give rise to flat conductors and shape conformable and flexible cables as seen in FIGURES 9-11. When plural laminations or strips are used, integration is effected in any manner and by suitable procedures. Specifically FIGURE 9 shows a single strip 145 in folded position and used as a single strip 145 in folded position and used as a single conductor; FIGURE 10 shows two strips 146 as two insulated conductors; and FIGURE 11 shows a plurality of strips 147 frictionally clamped by folding procedure herein to serve as a cable of more than two conductors. The folding procedure is best shown in FIGURE 19 as has been described.

#### Conclusion

This application is also an improvement over applicant's abandoned application for patent on Adhesive Conductors filed June 25, 1953 under Serial Number 364,112 and abandoned on November 9, 1957.

It is understood that in the interpretation of this specification, the separate description of each of the embodiments is not to be construed as mutually exclusive; applicable features, descriptive matter, structures and procedures of one or more embodiments alone or in various combinations form part of one or more of the other embodiments for purposes of either disclosing a completely operative structure, for additive combinations and for disclosure of equivalents. The foil of web 101a is to be considered as a reagent as well as the coating thereon for reaction chamber operation.

This interpretive consideration is expressed herein so that in the event of requirements for multiple division of the instant application, the full specification may be utilized for purposes of adequate disclosure to support true divisional cases of one or more embodiments from the parent case.

It is further understood that there may be minor changes and variations in the combinations, subcombinations, and individual assemblies and individual parts of the invention; in the combination, subcombination, individual and order of steps of the methods of the invention; in the integration of the assemblies and parts; in the sequences of operation and consolidation of assemblies and parts; in synchronization, power sources and connections. Variations depending upon requirements as to torque and temperature values, cubic feet of air per minute fed and exhausted, tension values, electrical power and kilocycles furnished, ultrasonic vibration values and dimensions and speed of parts are encompassed in the invention. There also may be minor changes and variations in the products disclosed as to size, shape, differential gauges, purposes, material and characteristics. All these changes and variations may be resorted to without departing from the spirit of the invention and the scope of the appended claims.

I claim:

1. In a method of coating metal foils, the steps comprising applying a polymerizable resinous coating to form a resin to one side of a travelling web of metallic foil of a gauge between .005 to .000175 inch to form a flexible electrical conductor and a dielectric non-strippably bonded thereto, heating said web and coating thereon during course of travel between 500° F. and 900° F. by air convection and radiation for softening the web and for curing the coating thereon, simultaneously and controllably stretching the web and coating thereon and simultaneously applying heated air streams to effect gaseous pressures at opposite faces of the web with greater pressure on the uncoated side for cushioning and maintaining the web against folding, wrinkling and displacement thereof and for pneumatic pressure wiping to insure uniform coating, taking up the slack of the web with coating thereon from said stretching, and annealing and orienting simultaneously by ambient air flow and said stretching the web and the coating to form a conductor having an annealed metallic foil component and a dielectric resin coating component bonded thereto and of uniform thicknesses and densities, said metallic foil being of non-magnetic and electrically conducting material and consisting of at least one metal selected from the group consisting of copper and aluminum.
2. In the method of claim 1 wherein the added step of guiding said uniform conductor along rollers is provided to prevent lateral strain, shift and shearing.

30

#### References Cited by the Examiner

##### UNITED STATES PATENTS

|           |       |               |       |           |
|-----------|-------|---------------|-------|-----------|
| 586,555   | 7/97  | Kelman        | ----- | 117-232   |
| 664,982   | 1/01  | Thornton      |       |           |
| 905,554   | 12/08 | Mitchell      | ----- | 174-119   |
| 1,149,599 | 8/15  | Small         | ----- | 339-198.1 |
| 1,835,002 | 12/31 | Birckmayer    | ----- | 153-2     |
| 2,075,906 | 4/37  | Maude         | ----- | 174-119   |
| 2,315,645 | 4/43  | Newton et al. | ----- | 117-231   |
| 2,327,048 | 8/43  | Joyce         | ----- | 339-198.1 |
| 2,328,096 | 8/43  | Reevely       | ----- | 117-65 X  |
| 2,383,964 | 9/45  | Grupe         | ----- | 117-7     |
| 2,561,982 | 7/51  | Hanna et al.  | ----- | 117-230   |
| 2,594,096 | 4/52  | Trigg         | ----- | 117-230   |
| 2,707,821 | 5/55  | Sowter        | ----- | 29-470.1  |
| 2,707,889 | 5/55  | Sowter        | ----- | 29-470.1  |
| 2,730,348 | 1/56  | Rendel        | ----- | 263-3     |
| 2,865,795 | 12/58 | Morrison      | ----- | 117-132 X |
| 2,890,874 | 6/59  | Peterson      | ----- | 263-3     |

WILLIAM D. MARTIN, Primary Examiner.

BENNETT G. MILLER, JOSEPH B. SPENCER,  
RICHARD D. NEVIUS, Examiners.